



US010232493B2

(12) **United States Patent**  
**Long et al.**

(10) **Patent No.:** **US 10,232,493 B2**  
(45) **Date of Patent:** **\*Mar. 19, 2019**

(54) **POLYCRYSTALLINE DIAMOND CUTTING ELEMENTS HAVING NON-CATALYST MATERIAL ADDITIONS**

(71) Applicant: **DIAMOND INNOVATIONS, INC.**,  
Worthington, OH (US)

(72) Inventors: **Christopher Allen Long**, Westerville,  
OH (US); **Andrew Gledhill**,  
Westerville, OH (US)

(73) Assignee: **Diamond Innovations, Inc.**,  
Worthington, OH (US)

(\*) Notice: Subject to any disclaimer, the term of this patent is extended or adjusted under 35 U.S.C. 154(b) by 451 days.

This patent is subject to a terminal disclaimer.

(21) Appl. No.: **14/707,289**

(22) Filed: **May 8, 2015**

(65) **Prior Publication Data**

US 2016/0325404 A1 Nov. 10, 2016

(51) **Int. Cl.**

**B24D 18/00** (2006.01)  
**B24D 3/06** (2006.01)  
**B22F 3/14** (2006.01)  
**B22F 7/06** (2006.01)  
**C22C 26/00** (2006.01)

(Continued)

(52) **U.S. Cl.**

CPC ..... **B24D 18/0009** (2013.01); **B22F 3/14** (2013.01); **B22F 7/06** (2013.01); **B24D 3/06** (2013.01); **C22C 26/00** (2013.01); **E21B 10/55** (2013.01); **E21B 10/567** (2013.01);  
(Continued)

(58) **Field of Classification Search**

CPC ... E21B 10/567; E21B 10/55; E21B 2010/545  
See application file for complete search history.

(56) **References Cited**

U.S. PATENT DOCUMENTS

4,518,659 A 5/1985 Gigl et al.  
9,476,258 B2 \* 10/2016 Gledhill ..... B24D 3/06  
(Continued)

FOREIGN PATENT DOCUMENTS

WO 2016118739 A1 7/2016

OTHER PUBLICATIONS

Schlumberger Oilfield Glossary entry for "PDC bit", accessed via [www.glossary.oilfield.slb.com](http://www.glossary.oilfield.slb.com).\*

*Primary Examiner* — Blake E Michener

(57) **ABSTRACT**

Polycrystalline diamond cutting elements having enhanced thermal stability, drill bits incorporating the same, and methods of making the same are disclosed herein. In one embodiment, a cutting element includes a substrate having a metal carbide and a polycrystalline diamond body bonded to the substrate. The polycrystalline diamond body includes a plurality of diamond grains bonded to adjacent diamond grains by diamond-to-diamond bonds and a plurality of interstitial regions positioned between adjacent diamond grains. At least a portion of the plurality of interstitial regions comprise a non-catalyst material, a catalyst material, metal carbide, or combinations thereof. At least a portion of the plurality of interstitial regions comprise non-catalyst material that coats portions of the adjacent diamond grains such that the non-catalyst material reduces contact between the diamond and the catalyst.

**26 Claims, 5 Drawing Sheets**  
**(2 of 5 Drawing Sheet(s) Filed in Color)**



(51) **Int. Cl.**  
*E21B 10/567* (2006.01)  
*E21B 10/55* (2006.01)  
*E21B 10/62* (2006.01)  
*E21B 10/54* (2006.01)  
*B22F 5/00* (2006.01)

(52) **U.S. Cl.**  
CPC .... *B22F 2005/001* (2013.01); *B22F 2999/00* (2013.01); *E21B 2010/545* (2013.01)

(56) **References Cited**

U.S. PATENT DOCUMENTS

9,920,578 B2 \* 3/2018 Gledhill ..... E21B 10/567  
2005/0230156 A1 \* 10/2005 Belnap ..... B22F 7/06  
175/375  
2010/0199573 A1 \* 8/2010 Montross ..... C22C 26/00  
51/307  
2011/0061942 A1 3/2011 Digiovanni  
2014/0318027 A1 10/2014 Mohammad  
2014/0360791 A1 \* 12/2014 Bowden ..... E21B 10/567  
175/432  
2014/0374172 A1 12/2014 Gledhill et al.  
2015/0367482 A1 \* 12/2015 Gledhill ..... B24D 3/10  
51/309  
2016/0326809 A1 \* 11/2016 Long ..... E21B 10/567

\* cited by examiner



FIG. 1



FIG. 2



FIG. 3



FIG. 4



**FIG. 5**





FIG. 7

## 1

**POLYCRYSTALLINE DIAMOND CUTTING  
ELEMENTS HAVING NON-CATALYST  
MATERIAL ADDITIONS**

**CROSS-REFERENCE TO RELATED  
APPLICATIONS**

None.

**TECHNICAL FIELD AND INDUSTRIAL  
APPLICABILITY**

The present disclosure relates generally to cutting elements made from superhard abrasive materials and, more particularly, to cutting elements made from polycrystalline diamond having a non-catalyst material addition that surround the individual diamond grains, and methods of making the same.

**BACKGROUND**

Polycrystalline diamond (“PCD”) compacts are used in a variety of mechanical applications, for example in material removal operations, as bearing surfaces, and in wire-drawing operations. PCD compacts are often used in the petroleum industry in the removal of material in downhole drilling. The PCD compacts are formed as cutting elements, a number of which are attached to drill bits, for example, roller-cone drill bits and fixed-cutting element drill bits.

PCD cutting elements typically include a superabrasive diamond layer, referred to as a polycrystalline diamond body, which is attached to a substrate. The polycrystalline diamond body may be formed in a high pressure high temperature (HPHT) process, in which diamond grains are held at pressures and temperatures to cause the diamond particles bond to one another.

As is conventionally known, the diamond particles are introduced to the HPHT process in the presence of a catalyst material that, when subjected to the conditions of the HPHT process, promotes formation of interparticle diamond bonds. The catalyst material may be embedded in a substrate, for example, a cemented tungsten carbide substrate having cobalt. The catalyst material may infiltrate the diamond particles from the substrate. Following the HPHT process, the diamond particles are sintered to one another and may be attached to the substrate.

While the catalyst material promotes formation of the inter-diamond bonds during the HPHT process, the presence of the catalyst material in the sintered diamond body after the completion of the HPHT process may also reduce the stability of the polycrystalline diamond body at elevated temperatures. Some of the diamond grains may undergo a back-conversion to a softer non-diamond form of carbon (for example, graphite or amorphous carbon) at elevated temperatures. Further, mismatch of the thermal expansion of the materials may induce stress into the diamond lattice causing microcracks in the diamond body. Back-conversion of diamond and stress induced by the mismatch of thermal expansion of the materials may contribute to a decrease in the toughness, abrasion resistance, and/or thermal stability of the PCD cutting elements during operation.

Accordingly, polycrystalline diamond cutting elements that have improved thermal stability may be desired.

**SUMMARY**

In one embodiment, a cutting element includes a substrate having a metal carbide and a polycrystalline diamond body

## 2

bonded to the substrate. The polycrystalline diamond body includes a plurality of diamond grains bonded to adjacent diamond grains by diamond-to-diamond bonds and a plurality of interstitial regions positioned between adjacent diamond grains. At least a portion of the plurality of interstitial regions include non-catalyst material having less than about 10 wt. % lead, a catalyst material, metal carbide, or combinations thereof. At least a portion of the plurality of interstitial regions include non-catalyst material that coats portions of the adjacent diamond grains such that the non-catalyst material reduces contact between the diamond and the catalyst.

In another embodiment, a polycrystalline diamond volume includes a plurality of diamond grains bonded to adjacent diamond grains by diamond-to-diamond bonds forming a continuous diamond matrix and a plurality of interstitial regions positioned between adjacent diamond grains and forming a continuous interstitial matrix. At least a portion of the continuous interstitial matrix includes catalyst material that is separated from the diamond grains by non-catalyst material having less than about 10 wt. % lead such that the non-catalyst material reduces contact between the diamond and the catalyst material.

In yet another embodiment, a cutting element includes a substrate that includes a metal carbide and a polycrystalline diamond body bonded to the substrate. The polycrystalline diamond body includes a plurality of diamond grains bonded to adjacent diamond grains by diamond-to-diamond bonds forming a continuous diamond matrix and a plurality of interstitial regions positioned between adjacent diamond grains and forming a continuous interstitial matrix. At least a portion of the continuous interstitial matrix includes catalyst material that is separated from the diamond grains by non-catalyst material having less than 10 wt. % lead, such that the non-catalyst material reduces contact between the diamond and the catalyst material.

In yet another embodiment, a method of forming a cutting element includes assembling a reaction cell comprising a plurality of diamond particles, non-catalyst material having less than about 10 wt. % lead, a catalyst material, and a substrate within a refractory metal container. The method further includes subjecting the reaction cell and its contents to a high pressure high temperature sintering process to form a continuous diamond volume. The diamond particles are compacted into a densified unbonded diamond region in which at least some of the diamond particles are separated by interstitial regions. The non-catalyst material is melted and is present in a liquid state in at least some of the interstitial regions between diamond particles. The catalyst material is melted and is present in at least some of the interstitial regions between the individual diamond grains, where the catalyst material promotes formation of diamond-to-diamond bonds between adjacent diamond particles. The non-catalyst material coats surfaces of at least a portion of the plurality of diamond particles after the high pressure high temperature sintering operation is completed.

In yet another embodiment, a drill bit includes a material removal portion having a plurality of shanks. The material removal portion having an axis of rotation that is relative to a base portion. The drill bit also includes at least one cutting element that is bonded to the material removal portion at one of the plurality of shanks. The cutting elements include a substrate comprising a metal carbide and a polycrystalline diamond body bonded to the substrate. The polycrystalline diamond body includes a plurality of diamond grains bonded to adjacent diamond grains by diamond-to-diamond bonds and a plurality of interstitial regions positioned between

adjacent diamond grains. At least a portion of the plurality of interstitial regions include non-catalyst material having less than about 10 wt. % lead, a catalyst material, metal carbide, or combinations thereof. At least a portion of the plurality of interstitial regions include non-catalyst material that coat portions of the adjacent diamond grains such that the non-catalyst material reduces contact between the diamond and the catalyst.

#### BRIEF DESCRIPTION OF THE DRAWINGS

The patent or application file contains at least one photomicrograph executed in color. Copies of this patent or patent application publication with color photomicrographs will be provided by the Office upon request and payment of the necessary fee.

The foregoing summary, as well as the following detailed description of the embodiments, will be better understood when read in conjunction with the appended drawings. It should be understood that the embodiments depicted are not limited to the precise arrangements and instrumentalities shown.

FIG. 1 is a schematic side cross-sectional view of a PCD cutting element according to one or more embodiments shown or described herein;

FIG. 2 is a detailed schematic side cross-sectional view of the PCD cutting element of FIG. 1A shown at location A;

FIG. 3 is a transmission electron micrograph of a cutting element according to one or more embodiments shown or described herein; and

FIG. 4 is a plot of energy dispersive X-ray spectroscopy for cobalt in the region of the cutting element depicted in FIG. 3;

FIG. 5 is a plot of energy dispersive X-ray spectroscopy for lead in the region of the cutting element depicted in FIG. 3;

FIG. 6 is a schematic flow chart depicting a manufacturing process of a PCD cutting element; and

FIG. 7 is a schematic perspective view of a drill bit having a plurality of PCD cutting elements according to one or more embodiments shown or described herein.

#### DETAILED DESCRIPTION

The present disclosure is directed to polycrystalline diamond cutting elements having enhanced thermal stability, drill bits incorporating the same, and methods of making the same. A cutting element may include a substrate and a polycrystalline diamond body bonded to the substrate. The polycrystalline diamond body may include a plurality of diamond grains bonded to adjacent diamond grains by diamond-to-diamond bonds and a plurality of interstitial regions positioned between adjacent diamond grains. At least a portion of the plurality of interstitial regions include a non-catalyst material that coats portions of the adjacent diamond grains such that the non-catalyst material reduces contact between the diamond and the catalyst introduced to aid in sintering of the diamond particles. Polycrystalline diamond cutting elements having enhanced thermal stability, drill bits incorporating the same, and methods of making the same are described in greater detail below.

It is to be understood that this disclosure is not limited to the particular methodologies, systems and materials described, as these may vary. It is also to be understood that the terminology used in the description is for the purpose of describing the particular versions or embodiments only, and is not intended to limit the scope. For example, as used

herein, the singular forms "a," "an," and "the" include plural references unless the context clearly dictates otherwise. In addition, the word "comprising" as used herein is intended to mean "including but not limited to." Unless defined otherwise, all technical and scientific terms used herein have the same meanings as commonly understood by one of ordinary skill in the art.

Unless otherwise indicated, all numbers expressing quantities of ingredients, properties such as size, weight, reaction conditions and so forth used in the specification and claims are to be understood as being modified in all instances by the term "about". Accordingly, unless indicated to the contrary, the numerical parameters set forth in the following specification and attached claims are approximations that may vary depending upon the desired properties sought to be obtained by the end user. At the very least, and not as an attempt to limit the application of the doctrine of equivalents to the scope of the claims, each numerical parameter should at least be construed in light of the number of reported significant digits and by applying ordinary rounding techniques.

As used herein, the term "about" means plus or minus 10% of the value of the number with which it is being used. Therefore, "about 40" means in the range of 36-44. As used herein, all numerical values should be interpreted to include "about" prior to their recitation.

Polycrystalline diamond compacts (or "PCD compacts", as used hereafter) may represent a volume of crystalline diamond grains with embedded non-diamond material filling the inter-granular spaces. In one example, a PCD compact includes a plurality of crystalline diamond grains that are bonded to each other by strong interparticle diamond bonds and forming a continuous polycrystalline diamond body, and the inter-granular regions, disposed between the bonded grains and filled with a non-diamond material (e.g., a catalyst material such as cobalt or its alloys), which was used to promote diamond bonding during fabrication of the PCD compact. Suitable metal solvent catalysts may include the metal in Group VIII of the Periodic table. Polycrystalline diamond cutting elements (or "PCD cutting element", as is used hereafter) include the above mentioned polycrystalline diamond body attached to a suitable substrate (for example, cemented tungsten carbide-cobalt (WC-Co)). The attachment between the polycrystalline diamond body and the substrate may be made by virtue of the presence of a catalyst, for example cobalt metal. In another embodiment, the polycrystalline diamond body may be attached to the substrate by brazing. In another embodiment, a PCD compact includes a plurality of crystalline diamond grains that are strongly bonded to each other by a hard amorphous carbon material, for example a-C or t-C carbon. In another embodiment, a PCD compact includes a plurality of crystalline diamond grains, which are not bonded to each other, but instead are bound together by foreign bonding materials such as borides, nitrides, or carbides, for example, SiC.

As used herein, the term "non-catalyst material" means any material that is non-catalytic with carbon-diamond conversion at elevated temperature.

As discussed above, conventional PCD cutting elements are used in a variety of industries and applications in material removal operations. PCD cutting elements are typically used in non-ferrous metal removal operations and in downhole drilling operations in the petroleum industry. Conventional PCD cutting elements exhibit high toughness, strength, and abrasion resistance because of the inter-granular inter-diamond bonding of the diamond grains that make up the polycrystalline diamond bodies of the PCD cutting

elements. The inter-diamond bonding of the diamond grains of the polycrystalline diamond body are promoted during an HPHT process by a catalyst material. However, at elevated temperature, the catalyst material and its byproducts that remain present in the polycrystalline diamond body after the HPHT process may promote back-conversion of diamond to non-diamond carbon forms and may induce stress into the diamond lattice due to the mismatch in the thermal expansion of the materials. The performance of the PCD cutting element at elevated temperature may be referred to as the "thermally stable" performance of the cutting element.

It is conventionally known to remove or deplete portions of the catalyst material to improve the thermal stability of the diamond body. The most common method of removing the catalyst material is a leaching process in which the PCD compact is introduced to a leaching agent, for example, an aqueous acid solution. The leaching agent may be selected from a variety of conventionally-known compositions in which the catalyst material is known to dissolve. By dissolving and removing at least a portion of the catalyst material from the PCD compact, the service life of the PCD compact may be increased due to the reduction in back-conversion rate of the diamond in the polycrystalline diamond body to non-diamond carbon forms and the reduction in materials having mismatched thermal expansion. However, a portion of catalyst material may still remain in the diamond body of the PCD compact that have been subjected to the leaching process. The interstitial regions between diamond grains may form "trapped" or "entrained" volumes into which the leaching agent has limited or no accessibility. Therefore, these trapped volumes remain populated with the constituents of the PCD formation process. The trapped volumes that contain catalyst material contribute to the degradation of the abrasion resistance of the PCD cutting element at elevated temperature that is generated during use of the PCD cutting element to remove material. Thus, reduction of trapped catalyst material may improve the abrasion resistance of PCD compact cutting elements.

The present disclosure is directed to polycrystalline diamond cutting elements that incorporate non-catalyst material that is distributed throughout the polycrystalline diamond body. Such non-catalyst materials may include metals, metal alloys, metalloids, semiconductors, and combinations thereof. Examples of such non-catalyst materials may include, for example and without limitation, copper, silver, gold, aluminum, silicon, gallium, tin, bismuth, indium, thallium, tellurium, antimony, polonium, lithium, magnesium, and alloys, carbides, nitrides, or carbonitrides thereof. In one embodiment, the non-catalyst material may be a non-catalyst material having less than about 10 wt. % lead. The non-catalyst material may be introduced to the diamond particles prior to or concurrently with the HPHT process. The non-catalyst material may be distributed throughout the polycrystalline diamond body evenly or unevenly, as well as by forming a distribution pattern. The non-catalyst material may reduce the amount of catalyst material that is present in the polycrystalline diamond body following the HPHT process. Further, the non-catalyst material may reduce the amount of catalyst material that is present in the polycrystalline diamond body following a leaching process in which at least portions of both the non-catalyst material and the catalyst material are removed from the interstitial regions of the polycrystalline diamond body. Additionally, the non-catalyst material may increase the removal rate (or the "leaching rate") of the catalyst material from the polycrystalline diamond body. In some embodiments, the non-catalyst material coats the diamond grains, thereby main-

taining a spacing between the catalyst material and the diamond grains for a plurality of diamond grains in the diamond body.

Because of the reduction of the catalyst material in the polycrystalline diamond body and because of the separation between the diamond grains and the catalyst material, polycrystalline diamond cutting elements according to the present disclosure exhibit performance that exceeds that of conventional PCD cutting elements in at least one of toughness, strength, and abrasion resistance.

Referring now to FIGS. 1 and 2, a PCD cutting element 100 is depicted. The PCD cutting element 100 includes a substrate 110 and a polycrystalline diamond body 120 that is attached to the substrate 110. The polycrystalline diamond body 120 includes a plurality of diamond grains 122 that are bonded to one another, including being bonded to one another through inter-diamond bonding. The bonded diamond grains 122 form a diamond lattice that extends along the polycrystalline diamond body 120. The diamond body 120 also includes a plurality of interstitial regions 124 between the diamond grains. The interstitial regions 124 represent a space between the diamond grains. In at least some of the interstitial regions 124, a non-carbon material is present. In some of the interstitial regions 124, non-catalyst material is present. In other interstitial regions 124, catalyst material is present. In yet other interstitial regions 124, both non-catalyst material and catalyst material are present. In yet other interstitial regions 124, at least one of catalyst material, non-catalyst material, swept material of the substrate 110, for example, cemented tungsten carbide, and reaction by-products of the HPHT process are present. Non-carbon, non-catalyst material, or catalyst materials may be bonded to diamond grains. Alternatively, non-carbon, non-catalyst material, or catalyst materials may be not bonded to diamond grains.

The catalyst material may be selected from a variety of materials that interact with the diamond particles to form interparticle diamond bonds. Examples of such materials include, for example and without limitation, elemental metallic catalyst such as elements selected from Group VIII of the periodic table, for example, cobalt, nickel, iron, or alloys thereof, as well as magnesium, chromium, tantalum, and niobium, metallic alloy catalysts selected Group IV, V, or VI of the periodic table alloyed with silver, copper, or gold, alkaline and alkaline earth compounds or carbonates thereof, and non-metallic elemental catalysts such as phosphorus and sulphur. The catalyst material may be present in a greater concentration in the substrate 110 than in the polycrystalline diamond body 120, and may promote attachment of the substrate 110 to the polycrystalline diamond body 120 in the HPHT process, as will be discussed below. The polycrystalline diamond body 120 may include an attachment region 128 that is rich in catalyst material promotes bonding between the polycrystalline diamond body 120 and the substrate 110. In other embodiments, the concentration of the catalyst material may be greater in the polycrystalline diamond body 120 than in the substrate 110. In yet other embodiments, the catalyst material may differ from the catalyst of the substrate 110. The catalyst material may be a metallic catalyst reaction-byproduct, for example catalyst-carbon, catalyst-tungsten, catalyst-chromium, or other catalyst compounds, which also may have lower catalytic activity towards diamond than a metallic catalyst.

The non-catalyst material may be selected from a variety of materials that are non-catalytic with the carbon-diamond conversion. The non-catalyst material may be generally immiscible with the catalyst material when both are liquid

such that the non-catalyst material and the catalyst material do not alloy with one another when both are liquid. In some embodiments, the non-catalyst material may have a lower liquidus or melting temperature than the liquidus or melting temperature of the catalyst material.

Both non-catalyst material and catalyst material may be present in a detectable amount in the polycrystalline diamond body of the PCD cutting element both before and after subjecting the polycrystalline diamond body to leaching. Presence of such materials may be identified by X-ray fluorescence, for example using a XRF analyzer available from Bruker AXS, Inc. of Madison, Wis., USA. Presence of such material may also be identified using X-ray diffraction, energy dispersive spectroscopy, or other suitable techniques.

The non-catalyst material may be introduced to the unbonded diamond particles prior to the HPHT process that bonds the diamonds particles in an amount that is in a range from about 0.1 vol. % to about 5 vol. % of the diamond body **120**, for example an amount that is in a range from about 0.2 vol. % to about 4 vol. % of the diamond body **120**, for example an amount that is in a range from about 0.5 vol. % to about 3 vol. %. In an exemplary embodiment, non-catalyst material may be introduced to the unbonded diamond in an amount from about 0.33 to about 1.5 vol. %. Following this HPHT process and leaching, the non-catalyst material content in the leached region of the diamond body **120** is reduced by at least about 50%, including being reduced in a range from about 50% to about 90%.

In the HPHT process that bonds the diamond particles, catalyst material may be introduced to the diamond powders. The catalyst material may be present in an amount that is in a range from about 0.1 vol. % to about 30 vol. % of the diamond body **120**, for example an amount that is in a range from about 0.3 vol. % to about 10 vol. % of the diamond body **120**, including being an amount of about 5 vol. % of the diamond body **120**. In an exemplary embodiment, catalyst material may be introduced to the unbonded diamond is an amount from about 4.5 vol. % to about 6 vol. %. Following this HPHT process and leaching, the catalyst material content in the leached region of the diamond body **120** is reduced by at least about 50%, including being reduced in a range from about 50% to about 90%.

The non-catalyst material and the catalyst material may be non-uniformly distributed in the bulk of the polycrystalline diamond cutting element **100** such that the respective concentrations of non-catalyst material and catalyst material vary at different positions within the polycrystalline diamond body **120**. In one embodiment the non-catalyst material may be arranged to have a concentration gradient that is evaluated along a longitudinal axis **102** of the polycrystalline diamond cutting element **100**. The concentration of the non-catalyst material may be higher at positions evaluated distally from the substrate **110** than at positions evaluated proximally to the substrate **110**. In opposite, the concentration of the catalyst material may be greater at positions evaluated proximally to the substrate **110** than at positions evaluated distally from the substrate **110**. In yet another embodiment, the concentrations of the non-catalyst material and the catalyst material may undergo a step change when evaluated in a longitudinal axis **192** of the polycrystalline diamond cutting element **100**. In yet another embodiment, the concentrations of the non-catalyst material and the catalyst material may exhibit a variety of patterns or configurations. Independent of the concentration of the non-catalyst material and the catalyst material in the polycrystalline diamond body **120**, however, both non-catalyst

material and catalyst material may be detectible along surfaces proximately and distally located relative to the substrate **110**.

In another embodiment, the polycrystalline diamond body **120** may exhibit relatively high amounts of the catalyst material at positions proximate to the substrate **110** and at which the catalyst material forms a bond between the polycrystalline diamond body **120** and the substrate **110**. In some embodiments, at positions outside of such an attachment zone, the non-catalyst material and the catalyst material maintain the concentration variation described above.

PCD cutting elements **100** according to the present disclosure may exhibit improved performance as compared to conventionally produced PCD cutting elements when evaluated in terms of abrasion resistance and/or toughness. The performance of PCD cutting elements **100** according to the present disclosure may particularly exhibit improved performance when subjected to conditions of elevated temperature. Such conditions may occur when the PCD cutting elements **100** are used in material removal operations, for example, downhole drilling operations in the petroleum industry. Performance of the PCD cutting element **100** with respect to abrasion resistance may be quantified in laboratory testing, for example using a simulated cutting operation in which the PCD cutting element **100** is used to machine an analogous material that replicates an end user application.

In one example used to replicate a downhole drilling application, the PCD cutting element **100** is held in a vertical turret lathe ("VTL") to machine granite. Parameters of the VTL test may be varied to replicate desired test conditions. In one example, the cutting element that is subjected to the VTL test is water cooled. In one example, the PCD cutting element **100** was positioned to maintain a depth of cut of about 0.017 inches/pass at a cross-feed rate of about 0.17 inches/revolution and a cutting element velocity of 122 surface feet per minute and a backrake angle of 15 degrees. The VTL test introduces a wear scar into the PCD cutting element **100** along the position of contact between the PCD cutting element **100** and the granite. The size of the wear scar is compared to the material removed from the granite to evaluate the abrasion resistance of the PCD cutting element **100**. The service life of the PCD cutting element **100** may be calculated based on the material removed from the granite as compared to the size of the wear scar abrades through the polycrystalline diamond body **120** and into the substrate **110**.

In another example, the PCD cutting element **100** is subjected to an interrupted milling test that implements a fly cutting tool holder and workpiece arrangement in which the PCD cutting element **100** is periodically removes material from a workpiece and then is brought out of contact with the workpiece. The interrupted milling test is described in U.S. patent application Ser. No. 13/791,277, the entire disclosure of which is hereby incorporated by reference. The interrupted milling test may evaluate thermal resistance of the PCD cutting element **100**.

In some embodiments, PCD cutting elements **100** according to the present disclosure exhibit increased abrasion resistance as compared to conventionally produced PCD cutting elements. In some embodiments, PCD cutting elements **100** according to the present disclosure may exhibit at least about 30% less wear with an equivalent amount of material removed from the granite as compared to conventionally produced PCD cutting elements, including exhibiting about 75% less wear than a conventional cutting element, including exhibiting about 90% less wear than a conventional cutting element.

PCD cutting elements 100 according to the present disclosure exhibit a lower concentration of catalyst material in trapped interstitial regions between the bonded diamond grains as compared to conventionally processed cutting elements. As discussed above, because the catalyst material that is positioned within the trapped interstitial regions may contribute to back-conversion of the diamond grains to non-diamond forms of carbon. The propensity of the polycrystalline diamond body 120 of the PCD cutting element 100 to back-convert to non-diamond forms of carbon and/or the stress induced to the polycrystalline diamond body 120 by the mismatch in thermal expansion of co joined material may be correlated to the high-temperature abrasion resistance of the PCD cutting element 100. Reducing the amount of the catalyst material within the trapped interstitial regions between diamond grains of the polycrystalline diamond body 120 may reduce the rate of back-conversion of the PCD cutting element 100. Further, reducing the amount of catalyst material within the trapped interstitial regions between diamond grains of the polycrystalline diamond body 120 may reduce stress that is induced into the diamond lattice caused by a mismatch in the thermal expansion of the diamond grains and the catalyst material. Therefore, the reduction in the catalyst material within the trapped interstitial regions between the diamond grains resulting from the introduction of non-catalyst material into the polycrystalline diamond body 120, improves performance of the PCD cutting element 100 as compared to conventionally produced PCD cutting elements.

Still referring to FIG. 1, some embodiments of the PCD cutting element 100 include a crown portion 402 that is positioned within the polycrystalline diamond body 120 and along a surface opposite the substrate 110. The crown portion 402 is made from a material that is dissimilar from the material of the polycrystalline diamond body 120 and the substrate 110. The crown portion 402 may extend into the diamond body 120 from the top surface of the PCD cutting element 100. The crown portion 402 may extend to a depth that is less than about 1 mm from the substrate 110 including being about 300  $\mu$ m from the substrate 110. The crown portion 402 may limit the depth that the catalyst material 94 sweeps into the polycrystalline diamond body 120 from the second substrate 110 during the second HPHT process. The crown portion 402 may provide locally modified material properties of the PCD cutting element 100. In one embodiment, the crown portion 402 may include, in addition to the bonded diamond grains and the non-catalyst material and the catalyst material in detectable amounts, a material selected from the group consisting of aluminum, aluminum carbide, silicon, and silicon carbide. In some embodiments, the polycrystalline diamond body 120 may be free of such materials outside of the attachment region 128.

PDC cutting elements according to the present disclosure may be fabricated using so-called "single press" or "double press" HPHT process. In a single press HPHT process, diamond particles may be subjected to a high pressure high temperature sintering process in which diamond particles are subjected to elevated pressure to form an unbonded diamond volume having a plurality of diamond particles that contact one another and a plurality of interstitial regions positioned between adjacent diamond particles. Non-catalyst material is melted and collects in interstitial regions. In some embodiments, the non-catalyst material may be mixed with the diamond particles prior to initiation of the HPHT process. In other embodiments, the non-catalyst material may be swept into the interstitial regions between the diamond particles during the HPHT process from an external source. In yet

other embodiments, the non-catalyst material may be both mixed with the diamond particles prior to initiation of the HPHT process and swept into the interstitial regions between the diamond particles during the HPHT process from an external source. The volume of non-catalyst material introduced to the diamond particles may be less than the total volume of the interstitial regions of the diamond region, such that the non-catalyst material present in the diamond volume cannot fill all of the interstitial regions between adjacent diamond grains.

Subsequent to melting of the non-catalyst material, the catalyst material may be melted. The non-catalyst material and the catalyst material may be selected such that the melting or liquidus temperature of the non-catalyst material is lower than the melting or liquidus temperature of the catalyst material. In some embodiments, the melting or liquidus temperature of the non-catalyst material may be lower than the solidus temperature of the catalyst material. In some embodiments, the catalyst material may be mixed with the diamond particles prior to initiation of the HPHT process. In other embodiments, the catalyst material may be swept into the interstitial regions between the diamond particles during the HPHT process from an external source, for example a substrate having a hard metal composition that includes a metal carbide and a catalyst material. In yet other embodiments, the catalyst material may be both mixed with the diamond particles prior to initiation of the HPHT process and swept into the interstitial regions between the diamond particles during the HPHT process from an external source. The components of the reaction cell may be maintained at a sintering temperature at which the diamond particles, aided by the catalyst material, form diamond-to-diamond bonds between adjacent diamond particles. In some embodiments, the non-catalyst material may exhibit a lower viscosity than the viscosity of the catalyst material at the sintering temperature of the HPHT process. The catalyst material may be forced through the interstitial regions between diamond particles by the elevated pressure at which the components of the reaction cell are held. The volume and composition of the catalyst material may displace portions of the non-catalyst material from the interstitial regions between diamond particles, thereby pushing non-catalyst material away from many surfaces of the diamond particles.

With the catalyst material molten in a liquid state, the catalyst may dissolve at least a portion of the carbon from the diamond particles. As is conventionally known, the molten catalyst material may act as a solvent catalyst that, when cooled, diamond may re-precipitate from, such that the diamond particles form diamond-to-diamond bonds between one another, thereby forming a polycrystalline diamond body. The polycrystalline diamond body includes a plurality of diamond grains that are coupled to one another through diamond-to-diamond bonds, and having a plurality of interstitial regions positioned therebetween. The diamond grains that are bonded to one another may form an interconnected continuous diamond matrix of diamond grains. Most of the interstitial regions between the diamond grains are connected to one another such that the interstitial regions form an interconnected continuous matrix of interstitial regions. However, some of the interstitial regions within the polycrystalline diamond body may be "trapped" such that they are separated from the interconnected continuous matrix of interstitial regions. The polycrystalline diamond body may be attached to a substrate. Following the HPHT process, the trapped interstitial regions and the continuous interstitial

## 11

matrix between the diamond grains may be filled with non-catalyst material, catalyst material, hard metal, or combinations thereof.

In such embodiments, the catalyst material that is present in the trapped interstitial regions and/or the continuous interstitial matrix may be spaced apart from the diamond grains in the continuous diamond matrix by the non-catalyst material. This result is surprising, because the catalyst material is generally better at "wetting" the surfaces of the diamond particles than any non-catalyst material that is present in the diamond region. Further, in embodiments according to the present disclosure, some surfaces of the diamond grains may be coated by the non-catalyst material, such that spacing between the diamond grains and the catalyst material is preserved following the HPHT process.

As conventionally known, the diamond body may be contacted with a leaching agent that removes at least a portion of the materials present in the interstitial regions that are positioned proximate to the location of leaching agent application. For example, the polycrystalline diamond body may be submerged in a leaching agent such that surfaces of the polycrystalline diamond body contact the leaching agent, while surfaces of the substrate, to which the polycrystalline diamond body are attached, are maintained spaced apart from contact with the leaching agent. The leaching agent may be selected to attack the non-catalyst material and the catalyst material while preserving the diamond grains.

The non-catalyst material and the catalyst material may undergo an oxidation-reduction reaction with the leaching agent. The non-catalyst material may be more reactive with the leaching agent than the catalyst material such that the rate of the leaching reaction per unit distance within the diamond body is faster for diamond bodies formed with non-catalyst material and catalyst material as compared to diamond bodies formed without the introduction of non-catalyst material. The non-catalyst material may exhibit a lower activation energy than the catalyst material with the leaching agent such that the rate of reaction is greater for the non-catalyst material than the catalyst material.

The incorporation of non-catalyst material into the diamond body during the HPHT process may result in a decrease in the total catalyst content both prior to and following leaching as compared to conventional cutting elements that do not include non-catalyst material. The decrease in catalyst content as compared to conventional cutting elements may increase cutting element life by decreasing internal mechanical stresses attributable to mismatch between the coefficients of thermal expansion and modulus of the diamond grains, the non-catalyst material, and the catalyst material, and any back-conversion to non-diamond forms of carbon, which may be accelerated due to the presence of catalyst material. Further, the increase in leaching rate may reduce manufacturing time associated with producing a cutting element according to embodiments disclosed herein, in particular, by reducing the cycle time associated with leaching the non-catalyst material and catalyst material from the interstitial regions of the diamond body.

Additionally, the incorporation of non-catalyst material into the diamond body during the HPHT process may result in a decrease in the hard metal concentration in the diamond body as compared to conventional diamond bodies made without the introduction of non-catalyst material. Hard metals are typically introduced to the diamond bodies during the HPHT process from the substrate. In one embodiment, the hard metal concentration within diamond bodies according to the present disclosure may be less than 70% of the

## 12

hard metal concentration of a conventional diamond body, for example being less than about 50% of the hard metal concentration of a conventional diamond body.

Further, the incorporation of the non-catalyst material to the polycrystalline diamond body may modify the microstructural configuration of the polycrystalline diamond body as compared to conventional polycrystalline diamond cutting elements. Referring now to FIG. 3, a transmission electron micrograph of the microstructure of a polycrystalline diamond cutting element that is manufactured according to the present disclosure is depicted. In this embodiment, non-catalyst material introduced as lead particles were mixed with the diamond particles prior to positioning the diamond particles in the refractory cup for manufacturing.

Lead particles were added at a concentration of about 0.5 wt. % of the lead-diamond mixture. The substrate included cemented tungsten carbide with about 12.5 wt. % cobalt, which acted as the catalyst in the HPHT process for sintering the diamond particles. The contents of the cell assembly used to manufacture the cutting element was subjected to a maximum temperature of about 1550° C. and a maximum pressure of 7.5 GPa, and were held above the melting temperature of cobalt for about 3 minutes. The PCD compact recovered from the HPHT process was further processed according to conventionally known procedures to a shape of a cutting element.

Following this processing, portions of the diamond volume were removed and prepared as a sample for the transmission electron microscopy. The sample of the diamond volume to be investigated was prepared using a dual beam focused ion beam ("FIB") to cut and extract a sufficiently thin section to allow for electron transmission. The sample was then examined in a transmission electron microscope ("TEM") at 200 kV.

The diamond grains (dark grey) are bonded to one another to form a continuous polycrystalline diamond matrix. The diamond volume also includes a continuous interstitial matrix (light grey) that is positioned between the diamond grains at positions spaced apart from the locations of diamond-to-diamond bonding. Note that the portion of the diamond volume from which the depicted sample has been taken from was unleached, such that none of the lead or lead alloy and catalyst material have been removed.

Referring to FIGS. 4 and 5, plots of energy dispersive X-ray spectroscopy data gathered from the location depicted in FIG. 3 are provided for lead in FIG. 4 and for catalyst material (here, cobalt) in FIG. 5. As can be seen in FIG. 4, a thin layer of lead or lead alloy coats portions of the diamond grains. In contrast, FIG. 5 depicts that cobalt fills the substantial majority of the remaining portions of the interstitial region.

The micrographs of FIGS. 4 and 5 indicate that there is a thin layer of lead or lead alloy that remains on some of the surfaces of the diamond grains following the HPHT process. The lead may be present along all of the surfaces of the diamond grain, but not visible in this sample configuration. Note that this lead or lead alloy remains present along the surfaces of the diamond grains following the HPHT process in which catalyst material is melted, molten catalyst material dissolves portions of the unbonded diamond particles, and the catalyst material solidifies and re-precipitates diamond at positions of diamond-to-diamond contact of the diamond grains in the presence of catalyst material.

In comparison to a conventional cutting element that does not include a non-catalyst material addition, it is believed that catalyst material remains present along the surfaces of the diamond grains following subjecting the cutting element to

## 13

a leaching process. Therefore, as compared to conventional cutting elements, cutting elements according to the present disclosure are believed to have lower catalyst content along the surfaces of the diamond grains. This reduction in catalyst content may reduce the total concentration of catalyst in the cutting element.

Further, the catalyst material positioned along surfaces of diamond grains of cutting elements according to the present disclosure may be functionally displaced by non-catalyst material. Without being bound by theory, the non-catalyst material does not have the same detrimental performance effects relating to the thermal stability of the diamond volumes on the cutting element when operating at elevated temperatures. Therefore, by incorporating the non-catalyst material along the surfaces of the diamond grain (and thereby displacing the catalyst material), the thermal stability of cutting elements according to the present disclosure may be enhanced as compared to conventional cutting elements that do not include a non-catalyst material addition.

In various embodiments, the non-catalyst material and the catalyst material may be selected based on the interactive properties of the non-catalyst material and the catalyst material. In one embodiment, the non-catalyst material may exhibit a melting or liquidus temperature that is lower than the melting or liquidus temperature of the catalyst material. In one embodiment, the non-catalyst material may be substantially immiscible with the catalyst material when both are in a liquid state. Such substantial immiscibility may be defined as less than about 10 at. % alloying of the materials. In one embodiment, the non-catalyst material may have greater than about 90 wt. % lead.

In one manufacturing process, cutting elements may be produced in a “single press” HPHT process in which diamond particles are bonded to one another and a substrate to form a cutting element having an integral diamond body with diamond grains bonded to one another in diamond-to-diamond bonds and interstitial regions between the diamond grains. Some of the interstitial regions include non-catalyst material, catalyst material, hard metal, or combinations thereof. Portions of the diamond body are maintained in contact with a leaching agent that removes substantially all of the non-catalyst material and catalyst material from a leached region positioned at the working surface of the cutting element and extending toward the substrate to a transition zone in which the leached region abuts the unleached region that is rich with non-catalyst material and catalyst material.

Referring now to FIG. 6, a flowchart depicting a manufacturing procedure 200 is provided. Diamond particles 90 are mixed with the non-catalyst material 92 in step 202. The size of the diamond particles 90 may be selected based on the desired mechanical properties of the polycrystalline diamond cutting element that is finally produced. It is generally believed that a decrease in grain size increases the abrasion resistance of the polycrystalline diamond cutting element, but decreases the toughness of the polycrystalline diamond cutting element. Further, it is generally believed that a decrease in grain size results in an increase in interstitial volume of the PCD compact. In one embodiment, the diamond particles 90 may have a single mode median volumetric particle size distribution (D50) in a range from about 10  $\mu\text{m}$  to about 100  $\mu\text{m}$ , for example having a D50 in a range from about 14  $\mu\text{m}$  to about 50  $\mu\text{m}$ , for example having a D50 of about 30  $\mu\text{m}$  to about 32  $\mu\text{m}$ . In other embodiments, the diamond particles 90 may have a D50 of about 14  $\mu\text{m}$ , or about 17  $\mu\text{m}$ , or about 30  $\mu\text{m}$ , or about 32

## 14

$\mu\text{m}$ . In other embodiments, the diamond particles 90 may have a multimodal particle size, wherein the diamond particles 90 are selected from two or more single mode populations having different values of D50, including multimodal distributions having two, three, or four different values of D50.

The non-catalyst material 92 may be introduced to step 402 as a powder. In other embodiments, the non-catalyst material 92 may be coated onto the unbonded diamond particles. The particle size of the non-catalyst material may be in a range from about 0.005  $\mu\text{m}$  to about 100  $\mu\text{m}$ , for example being in a range from about 10  $\mu\text{m}$  to about 50  $\mu\text{m}$ .

The diamond particles 90 and the non-catalyst material 92 may be dry mixed with one another using, for example, a commercial TURBULA® Shaker-Mixer available from Glen Mills, Inc. of Clifton, N.J. or an acoustic mixer available from Resodyn Acoustic Mixers, Inc. of Butte, Mont. to provide a generally uniform and well mixed combination. In other embodiments, the mixing particles may be placed inside a bag or container and held under vacuum or in a protective atmosphere during the blending process.

In other embodiments, the non-catalyst material 92 may be positioned separately from the diamond particles 90. During the first HPHT process, the non-catalyst material 92 may “sweep” from their original location and through the diamond particles 90, thereby positioning the non-catalyst material 92 prior to sintering of the diamond particles 90. Subsequent to sweeping of the non-catalyst material 92, the catalyst material 94 may be swept through the diamond particles 90 during the first HPHT process, thereby promoting formation of inter-diamond bonds between the diamond particles 90 and sintering of the diamond particles 90 to form the polycrystalline diamond body 120 of the polycrystalline diamond compact 80.

The diamond particles 90 and the non-catalyst material 92 may be positioned within a cup 142 that is made of a refractory material, for example tantalum, niobium, vanadium, molybdenum, tungsten, or zirconium, as shown in step 204. The substrate 110 is positioned along an open end of the cup 142 and is optionally welded to the cup 142 to form cell assembly 140 that encloses diamond particles 90 and the non-catalyst material 92. The substrate 110 may be selected from a variety of hard phase materials having metal carbides including, for example, cemented tungsten carbide, cemented tantalum carbide, or cemented titanium carbide. In one embodiment, the substrate 110 may include cemented tungsten carbide having free carbons, as described in U.S. Provisional Application Nos. 62/055,673, 62/055,677, and 62/055,679, the entire disclosures of which are hereby incorporated by reference. The substrate 110 may include a pre-determined quantity of catalyst material 94. Using a cemented tungsten carbide-cobalt system as an example, the cobalt is the catalyst material 94 that is infiltrated into the diamond particles 90 during the HPHT process. In other embodiments, the cell assembly 140 may include additional catalyst material (not shown) that is positioned between the substrate 110 and the diamond particles 90. In further other embodiments, the cell assembly 140 may include non-catalyst material 92 that is positioned between the diamond particles 90 and the substrate 110 or between the diamond particles 90 and the additional catalyst material (not shown).

The cell assembly 140, which includes the diamond particles 90, the non-catalyst material 92, and the substrate 110, is introduced to a press that is capable of and adapted to introduce ultra-high pressures and elevated temperatures to the cell assembly 140 in an HPHT process, as shown in

step 208. The press type may be a belt press, a cubic press, or other suitable presses. The pressures and temperatures of the HPHT process that are introduced to the cell assembly 140 are transferred to contents of the cell assembly 140. In particular, the HPHT process introduces pressure and temperature conditions to the diamond particles 90 at which diamond is stable and inter-diamond bonds form. The temperature of the HPHT process may be at least about 1000° C. (e.g., about 1200° C. to about 1800° C., or about 1300° C. to about 1600° C.) and the pressure of the HPHT process may be at least 4.0 GPa (e.g., about 4.0 GPa to about 12.0 GPa, or about 5.0 GPa to about 10 GPa, or about 5.0 GPa to about 8.0 GPa) for a time sufficient for adjacent diamond particles 90 to bond to one another, thereby forming an integral PCD compact having the polycrystalline diamond body 120 and the substrate 110 that are bonded to one another.

An integral PCD compact 82 having a polycrystalline diamond body 120 that is bonded to the substrate 110 may be recovered from the HPHT cell, as depicted in step 210. The introduction of the non-catalyst material 92 to the polycrystalline diamond body 120 prior to the HPHT process may result in a reduction of catalyst material 94 that is present in the polycrystalline diamond body 120 following the HPHT process and prior to initiation of any subsequent leaching process. As compared to conventional cutting elements that are produced without the introduction of the non-catalyst material 92, unleached diamond bodies 120 produced according to the present disclosure may contain, for example, about 10% less catalyst material 94 when evaluated prior to leaching.

The polycrystalline diamond body 120 may undergo a leaching process in which the catalyst material is removed from the polycrystalline diamond body 120. In one example of a leaching process, the polycrystalline diamond body 120 is introduced to a leaching agent of an acid bath to remove the remaining substrate 110 from the polycrystalline diamond body 120, as shown in step 212. The leaching process may also remove non-catalyst material 92 and catalyst material 94 from the polycrystalline diamond body 120 that is accessible to the acid. Suitable acids may be selected based on the solubility of the non-catalyst material 92 and the catalyst material 94 that is present in the polycrystalline diamond body. Examples of such acids including, for example and without limitation, ferric chloride, cupric chloride, nitric acid, hydrochloric acid, hydrofluoric acid, aqua regia, or solutions or mixtures thereof. The acid bath may be maintained at an pre-selected temperature to modify the rate of removal of the non-catalyst material 92 and the catalyst material 94 from the polycrystalline diamond body 120, including being in a temperature range from about 10° C. to about the boiling point of the leaching agent. In some embodiments, the acid bath may be maintained at elevated pressures that increase the liquid boiling temperature and thus allow the use of elevated temperatures, for example being at a temperature of greater than the boiling point of the leaching agent at atmospheric pressure. The polycrystalline diamond body 120 may be subjected to the leaching process for a time sufficient to remove the desired quantity of non-catalyst material 92 and catalyst material 94 from the polycrystalline diamond body. The polycrystalline diamond body 120 may be subjected to the leaching process for a time that ranges from about one hour to about one month, including ranging from about one day to about 7 days.

In some embodiments, the polycrystalline diamond body 120 may be maintained in the leaching process until the polycrystalline diamond body 120 is at least partially

leached. In polycrystalline diamond bodies 120 that are partially leached, the exterior regions of the polycrystalline diamond bodies 120 that are positioned along the outer surfaces of the polycrystalline diamond bodies 120 have the accessible interstitial regions depleted of non-catalyst material 92 and/or catalyst material 94, while the interior regions of the polycrystalline diamond bodies 120 are rich with non-catalyst material 92 and/or catalyst material 94. In such partially leached polycrystalline diamond bodies 120, all of the accessible interstitial regions between the diamond grains may be fully depleted of non-catalyst material 92 and/or catalyst material 94. In some embodiments, hard metal that is introduced to the polycrystalline diamond body 120 during the HPHT process may remain in the accessible interstitial regions.

In some embodiments, the extent of the leaching may be monitored by weighing the polycrystalline diamond body 120 after a pre-defined period of time. As the change in the weight loss of the polycrystalline diamond body 120 approaches a threshold value (for example, 10% loss of the unleached polycrystalline diamond body 120), the polycrystalline diamond body 120 may be considered to be completely leached. Because the polycrystalline diamond body 120 is leached without the substrate 110, the leach fronts may extend from opposing sides of the polycrystalline diamond body 120 and from the perimeter surface of the polycrystalline diamond body 120. When the leach fronts from the opposing sides of the polycrystalline diamond body 120 meet, the polycrystalline diamond body 120 may be considered to be completely leached. In some embodiments, the extent of leaching may be monitored by the loss of density of the diamond body.

In some embodiments, an unleached polycrystalline diamond body may have non-catalyst material 92 and catalyst material 94 at greater than about 4 vol. % of the polycrystalline diamond body 120, including being from about 4 vol. % to about 15 vol. %. In comparison, a completely leached portion of a polycrystalline diamond body 120 may have non-catalyst material 92 and catalyst material 94 that is less than about 80% less than the unleached polycrystalline diamond body 120, for example being in a range from about 60% to about 80% less than the unleached polycrystalline diamond body 120. A completely leached polycrystalline diamond body 120 may have non-catalyst material 92 and catalyst material 94 being from about 0.25 vol. % to about 6 vol. %, for example, being from about 0.2 vol. % to about 1 vol. %. In general, the extent of loss of non-catalyst material and catalyst material in a completely leached polycrystalline diamond body 120 is determined the material structure and composition, for example by the precursor diamond grain size and the particle size distribution.

As discussed above, the introduction of the non-catalyst material to the polycrystalline diamond body 120 reduces the concentration of the catalyst material 94 in the polycrystalline diamond body 120 prior to any leaching process. Further, subsequent to leaching regions of the polycrystalline diamond body 120, the introduction of the non-catalyst material 92 to the polycrystalline diamond body 120 also reduces the concentration of the catalyst material 94 that remains present in the trapped interstitial volumes of the polycrystalline diamond body 120 of the leached region of the polycrystalline diamond body 120. As compared to conventional cutting elements that are produced without the introduction of the non-catalyst material 92, diamond bodies 120 produced according to the present disclosure contain

from about 30 vol. % to about 90 vol. % less catalyst material **94** following complete leaching of both of the compared diamond bodies.

The introduction of the non-catalyst material **92** to the polycrystalline diamond body **120** may also increase the leaching rate of the polycrystalline diamond body **120**, such that the duration of time required to obtain complete leaching of the polycrystalline diamond body **120** is reduced as compared to conventionally produced diamond bodies. For example, complete leaching of the polycrystalline diamond body **120** having non-catalyst material **92** according to the present disclosure may be obtained from about 30% to about 60% less time as compared to conventional cutting elements that are produced without the introduction of the non-catalyst material **92**. In one example, when evaluated after 7 days of introduction to the leaching process, polycrystalline diamond bodies **120** produced according to the present disclosure exhibited from about 40% to about 70% more mass loss than conventional PCD compacts.

Following substantially complete leaching of the polycrystalline diamond body **120**, the polycrystalline diamond body **120** continues to exhibit non-diamond components that are present in the trapped interstitial regions of the polycrystalline diamond body **120** that are positioned between bonded diamond grains in at least detectable amounts. However, the reduction of the non-diamond components (including catalyst material **94**) in the leaching process accessible interstitial regions reduces the content of catalyst material **94** in the polycrystalline diamond body **120** and increases the thermal stability of the polycrystalline diamond body **120**.

Following formation of the integral PCD compact **82**, the PCD compact **82** may be processed through a variety of finishing operations to remove excess material from the PCD compact **82** and configure the PCD compact **82** for use by an end user, including formation of a cutting element **84**, as shown in step **418**. Such finishing operations may include, for example, grinding and polishing the outside diameter of the PCD compact **82**, cutting, grinding, lapping, and polishing the opposing faces (both the support-substrate-side face and the diamond-body-side face) of the PCD compact **82**, and grinding and lapping a chamfer into the PCD compact **82** between the diamond-body-side face and the outer diameter of the PCD compact **82**.

In an alternative manufacturing process, cutting elements may be produced in a “double press” HPHT process in which diamond particles are bonded to one another to form the diamond body in a first HPHT process, the diamond body is fully leached of non-catalyst material and catalyst material from the interstitial regions between the diamond grains, and the diamond body is attached to a substrate in a second HPHT process. The diamond particles may first be subjected to a first HPHT process to form a polycrystalline diamond compact having a polycrystalline diamond body that is formed through sintering with a catalyst material source. In one embodiment, the catalyst material source is provided integrally with a substrate (a first substrate). Substantially all of the substrate is removed from the polycrystalline diamond body, the polycrystalline diamond body is machined to a desired shape, and the polycrystalline diamond body is leached to remove substantially all of the accessible non-catalyst material and catalyst material from the interstitial regions of the polycrystalline diamond body. The leached polycrystalline diamond body is subsequently cleaned of leaching debris and bonded to a substrate in a second HPHT process, thus forming a PCD compact. This PCD compact is subsequently finished according to conven-

tionally known procedures to the final shape desirable of the PCD cutting elements for the end user application.

Referring now to FIG. 7, a plurality of PCD cutting elements **100** according to the present disclosure may be installed in a drill bit **310**, as conventionally known, to perform a downhole drilling operation. The drill bit **310** may be positioned on a drilling assembly **300** that includes a drilling motor **302** that applies torque to the drill bit **310** and an axial drive mechanism **304** that is coupled to the drilling assembly for moving the drilling assembly **300** through a borehole **60** and operable to modify the axial force applied by the drill bit **310** in the borehole **60**. Force applied to the drill bit **310** is referred to as “Weight on Bit” (“WOB”). The drilling assembly **300** may also include a steering mechanism that modifies the axial orientation of the drill assembly **300**, such that the drill bit **310** can be positioned for non-linear downhole drilling.

The drill bit **310** includes a stationary portion **312** and a material removal portion **314**. The material removal portion **314** may rotate relative to the stationary portion **312**. Torque applied by the drilling motor **302** rotates the material removal portion **314** relative to the stationary portion **312**. A plurality of PCD cutting elements **100** according to the present disclosure are coupled to the material removal portion **314**. The plurality of PCD cutting elements **100** may be coupled to the material removal portion **314** by a variety of conventionally known methods, including attaching the plurality of PCD cutting elements **100** to a corresponding plurality of shanks **316** that are coupled to the material removal portion **314**. The PCD cutting elements **100** may be coupled to the plurality of shanks **316** by a variety of methods, including, for example, brazing, adhesive bonding, or mechanical affixation. In embodiments in which the PCD cutting elements **100** are brazed to the shanks **316** with a braze filler **318**, at least a portion of the shanks **316**, the braze filler **318**, and at least a portion of the substrate **110** of the PCD cutting elements **100** is heated to an elevated temperature while in contact with one another. As the components decrease in temperature, the braze filler **318** solidifies and forms a bond between the substrate **110** of the PCD cutting elements **100** and the shanks **316** of the material removal portion **314**. In one embodiment, the brazing filler **318** has a melting temperature that is greater than a melting temperature of the non-catalyst material **92** of the polycrystalline diamond body **120** at ambient pressure conditions. In another embodiment, the brazing filler **318** has a melting temperature that is less than the catalyst material **94** of the polycrystalline diamond body **120** at ambient pressure conditions. In yet another embodiment, the brazing filler **318** has a melting temperature that is less than the liquidus temperature of the catalyst material **94** of the polycrystalline diamond body at ambient pressure conditions.

When the drill bit **310** is positioned in the borehole **60**, the material removal portion **314** rotates about the stationary portion **312** to reposition the PCD cutting elements **100** relative to the borehole **60**, thereby removing surrounding material from the borehole **60**. Force is applied to the drill bit **310** by the axial drive mechanism **304** in generally the axial orientation of the drill bit **310**. The axial drive mechanism **304** may increase the WOB, thereby increasing the contact force between the PCD cutting elements **100** and the material of the borehole **60**. As the material removal portion **314** of the drill bit **310** continues to rotate and WOB is maintained on the drill bit **310**, the PCD cutting elements **100** abrade material of the borehole **60**, and continue the path of the borehole **60** in an orientation that generally corresponds to the axial direction of the drill bit **310**.

19

It should now be understood that PCD cutting elements according to the present disclosure include a non-catalyst material addition to the diamond volume that is positioned within interstitial regions between adjacent diamond grains. The non-catalyst material may reduce contact between the diamond grains and a catalyst material that the diamond grains dissolve into when the catalyst material is molten. By preserving spacing between the catalyst material and the diamond grains, the PCD cutting element may exhibit improved performance at elevated temperatures as compared to conventional PCD cutting elements.

The invention claimed is:

1. A cutting element, comprising:

a substrate comprising a metal carbide; and  
a polycrystalline diamond body bonded to the substrate, 15  
the polycrystalline diamond body comprising a plurality of diamond grains bonded to adjacent diamond grains by diamond-to-diamond bonds and a plurality of interstitial regions positioned between adjacent diamond grains,

wherein at least a portion of the plurality of interstitial regions comprises a non-catalyst material having more than 0.1 wt % lead and having less than about 10 wt. % lead, which coats portions of the adjacent diamond and reduces contact between the diamond and a catalyst. 20

2. The cutting element of claim 1, wherein at least a portion of the plurality of interstitial regions are substantially free of non-catalyst material and catalyst material.

3. The cutting element of claim 2, wherein the portion of the plurality of interstitial regions that are substantially free of non-catalyst material and catalyst material are subject to a leaching process. 30

4. The cutting element of claim 1, wherein portions of the catalyst material that is positioned within the interstitial regions are spaced apart from the diamond grains by the non-catalyst material. 35

5. The cutting element of claim 1, wherein the diamond grains have higher wettability with the catalyst material than the non-catalyst material when both are molten.

6. The cutting element of claim 1, wherein when the non-catalyst material and the catalyst material are held at a temperature above the melting or liquid temperature of the catalyst material, the non-catalyst material has a lower viscosity than the catalyst material. 40

7. The cutting element of claim 1 wherein the plurality of interstitial regions comprises a non-catalyst material having more than 0.1 wt % lead and having less than 3.0 wt % of lead. 45

8. The cutting element of claim 1 wherein the plurality of interstitial regions comprises a non-catalyst material having more than 0.1 wt % lead and having less than 1.0 wt % of lead. 50

9. The cutting element of claim 1 wherein the plurality of interstitial regions comprises a non-catalyst material having more than about 1.0 wt % of lead and less than about 3.0 wt % of lead. 55

10. A polycrystalline diamond volume comprising:  
a plurality of diamond grains bonded to adjacent diamond grains by diamond-to-diamond bonds forming a continuous diamond matrix and a plurality of interstitial regions positioned between adjacent diamond grains and forming a continuous interstitial matrix, 60

wherein at least a portion of the continuous interstitial matrix comprises a catalyst material that is separated from the diamond grains by a non-catalyst material, wherein the non-catalyst material has more than 0.1 wt % lead and has less than about 10 wt. % lead, and

20

wherein the non-catalyst material coats portions of the diamond grains such that the non-catalyst material reduces contact between the diamond grains and the catalyst material.

5 11. The cutting element of claim 10, wherein at least a portion of the plurality of interstitial regions are substantially free of the non-catalyst material and the catalyst material.

12. The cutting element of claim 11, wherein the portion of the plurality of interstitial regions that are substantially free of the non-catalyst material and the catalyst material were subjected to a leaching process.

13. The cutting element of claim 10, wherein the diamond grains have higher wettability with the catalyst material than the non-catalyst material when both are molten.

14. A cutting element comprising:

a substrate comprising a metal carbide; and  
a polycrystalline diamond body bonded to the substrate, 20  
the polycrystalline diamond body comprising a plurality of diamond grains bonded to adjacent diamond grains by diamond-to-diamond bonds forming a continuous diamond matrix and a plurality of interstitial regions positioned between adjacent diamond grains and forming a continuous interstitial matrix,

wherein at least a portion of the continuous interstitial matrix comprises a catalyst material that is separated from the diamond grains by a non-catalyst material, wherein the non-catalyst material has more than 0.1 wt % lead and has less than about 10 wt. % lead, and wherein the non-catalyst material coats portions of the diamond grains such that the non-catalyst material reduces contact between the diamond grains and the catalyst material.

15. A method of forming a cutting element, comprising:  
assembling a reaction cell comprising a plurality of diamond particles, a non-catalyst material having more than 0.1 wt % lead and less than about 10 wt % lead, a catalyst material, and a substrate within a refractory metal container; and  
subjecting the reaction cell and its contents to a high pressure high temperature sintering process to form a continuous diamond volume in which:

the diamond particles are compacted into a densified unbonded diamond region in which at least some of the diamond particles are separated by interstitial regions;

the non-catalyst material is melted and is present in a liquid state in at least some of the interstitial regions between diamond particles; and  
the catalyst material is melted and is present in at least some of the interstitial regions between the individual diamond grains, wherein the catalyst material promotes formation of diamond-to-diamond bonds between adjacent diamond particles,

wherein the non-catalyst material coats surfaces of at least a portion of the plurality of diamond particles after the high pressure high temperature sintering operation is completed such that the non-catalyst material reduces contact between the diamond grains and the catalyst material.

16. The method of claim 15, wherein the catalyst material is swept through at least a portion of the plurality of unbonded diamond particles while molten and displaces a portion of the non-catalyst material from the interstitial regions between diamond particles. 65

**21**

17. The method of claim 15, wherein the non-catalyst material is swept through at least a portion of the plurality of unbonded diamond particles while molten.

18. The method of claim 15, wherein the non-catalyst material is mixed with the diamond particles prior to the step 5 of compaction of the diamond particles.

19. The method of claim 15, wherein the volume of non-catalyst material introduced to the diamond particles is less than a volume of interstitial regions between diamond particles.

20. The method of claim 15, wherein when the non-catalyst material and the catalyst material are held at a temperature above the melting or liquid temperature of the catalyst material, the non-catalyst material has a lower viscosity than the catalyst material.

21. The method of claim 15, further comprising subjecting the diamond volume to a leaching process in which a leaching agent removes at least portions of the catalyst material and non-catalyst material from the interstitial regions of the diamond volume.

22. The method of claim 15, wherein the diamond grains have higher wettability with the catalyst material than the non-catalyst material when both are molten.

23. A drill bit comprising:

a material removal portion having a plurality of shanks, the material removal portion having an axis of rotation that is relative to a base portion; and

**22**

at least one cutting element that is bonded to the material removal portion at one of the plurality of shanks, the cutting elements comprising:

a substrate comprising a metal carbide; and a polycrystalline diamond body bonded to the substrate, the polycrystalline diamond body comprising a plurality of diamond grains bonded to adjacent diamond grains by diamond-to-diamond bonds and a plurality of interstitial regions positioned between adjacent diamond grains,

wherein at least a portion of the plurality of interstitial regions comprise non-catalyst material having more than 0.1 wt % lead and less than about 10 wt. % lead, which coats portions of the adjacent grains and reduces contact between the diamond and a catalyst material.

24. The cutting element of claim 23 wherein the plurality of interstitial regions comprises a non-catalyst material having more than 0.1 wt % lead and having less than 3.0 wt % of lead.

25. The cutting element of claim 23 wherein the plurality of interstitial regions comprises a non-catalyst material having more than 0.1 wt % lead and having less than 1.0 wt % of lead.

26. The cutting element of claim 23 wherein the plurality of interstitial regions comprises a non-catalyst material having about 1.0 wt % of lead.

\* \* \* \* \*